

## UNITED STATES PATENT OFFICE

2,452,319

RUST AND OXIDATION INHIBITED  
LUBRICATING COMPOSITIONS

John A. Patterson and Herman D. Kluge, Beacon,  
N. Y., assignors to The Texas Company, New  
York, N. Y., a corporation of Delaware

No Drawing. Application December 8, 1943,  
Serial No. 513,466

4 Claims. (Cl. 252—49.6)

1

This invention relates to an improved lubricating composition and particularly to an oxidation inhibited hydrocarbon oil which is rendered rust-proof in the presence of water by the incorporation of a novel combination of addition agents.

Hydrocarbon oils used in lubricating compositions are usually subject to deterioration caused by heat and aeration resulting from the conditions of operation of the lubricant. This deterioration or oxidation causes the formation of acidic and sludge-like bodies which attack the bearing metals and deposit carbonaceous films on the surfaces to be lubricated. These deleterious effects have been substantially reduced by the incorporation of small amounts of so-called oxidation inhibitors which retard or minimize the formation of these acidic and sludge-like bodies in the oil.

Such inhibited lubricants have given satisfactory service in the lubrication of dry systems, but an added problem is encountered in lubricating systems where small amounts of water may accumulate. It has been found that such conditions of lubrication cause rusting or corrosion of the metal surfaces which results in uneven lubrication, increased wear and possible seizure between parts of narrow clearances due to the sloughing-off of rust particles and entrainment thereof in the lubricant body. This is particularly noticeable in the lubrication of steam-driven or marine equipment where leakage and steam condensation can hardly be avoided. To a lesser extent, rusting or corrosion is obtained in the lubrication of metal surfaces exposed to humid atmospheric conditions, such as textile and other industrial equipment, or in the lubrication of enclosed systems which are subject to intermittent operation, such as internal combustion engines, railway equipment, etc., which allow condensation within the system or parts thereof during the standing periods.

It is the purpose of this invention to provide a lubricating composition which possesses both rust-proof and oxidation-resistant properties and also a method of inhibiting oxidation-resistant lubricants so as to minimize the formation of rust or corrosion upon metallic surfaces lubricated thereby in the presence of water.

In accordance with the present invention it has been discovered that an oxidation-inhibited lubricating composition may be rendered rust-proof by the incorporation of small amounts of an additive composition consisting of a combination of an oil-miscible dicarboxylic acid and an oil-miscible organic acid ester of an acid of phosphorus.

2

It has also been discovered that a hydrocarbon oil, such as a mineral lubricating oil, which is compounded with an oxidation inhibitor and the combination of a dicarboxylic acid and an organic acid ester of an acid of phosphorus, possesses greater oxidation-resistant properties than are obtained with the oxidation inhibitor, per se.

The oxidation inhibitors which may be used in conjunction with the combination of the dicarboxylic acid and the organic acid ester of an acid of phosphorus are those which normally provide a resistance to oxidation when compounded with a hydrocarbon oil or lubricating composition subject to operation in the presence of water. These inhibitors are usually water-insoluble and resistant to hydrolysis or decomposition in the presence of water. Compounds of this nature, which are effective anti-oxidants in the presence of water, may be generally classified into three types of compounds, namely N-substituted aromatic amines, aromatic hydroxy compounds, and sulfur-containing compounds. The amounts in which these inhibitors are incorporated in a hydrocarbon oil or lubricating composition are usually within the range of 0.01-5.0% by weight and, in most instances, between 0.1-2.0% by weight.

It has been found that by incorporating an additive composition consisting of a combination of an oil-miscible dicarboxylic acid and an oil-miscible organic acid ester of an acid of phosphorus in an oxidation-inhibited hydrocarbon oil or a lubricating composition, a compounded lubricant is obtained which possesses both rust-inhibiting properties and enhanced anti-oxidant properties.

The sequence of incorporation is not a limitation of the present invention and the various addition agents may be incorporated as a unit or 40 each individual component may be incorporated separately. The practical aspects of the method of incorporation depend entirely upon the compatibility of the particular compounds selected.

The combination of the oil-miscible dicarboxylic acid and the organic acid ester of the acid of phosphorus is described and claimed in copending application serial No. 762,008 filed July 18, 1947, as a continuation of Serial No. 509,122 (now abandoned), filed November 5, 1943. The combination of an oil-miscible dicarboxylic acid and a diamino diaryl alkane in a lubricating composition, is described and claimed in our copending application Serial No. 632,106, filed November 30, 1945 as a continuation-in-part of Serial No. 519,558 (abandoned), filed January 26, 1944. The

disclosures thereof are directed to the rust-preventive properties and anti-oxidant properties of the respective additive compositions when applied to metallic surfaces exposed to water and other corrosive bodies conducive to the formation of rust. For the purposes of this invention the dicarboxylic acid component of the combination may be any dicarboxylic acid which contains at least 10 carbon atoms in the molecule and at least one carbon atom between the carboxyl groups; such acids include the derivatives of aromatic dicarboxylic acids, cycloaliphatic dicarboxylic acids and aliphatic dicarboxylic acids.

All dicarboxylic acids may be considered as being classified in either of two groups: (1) dicarboxylic acids which exist in stereo-isomeric form; and (2) dicarboxylic acids which possess a fixed configuration. It has been found that the greatest rust protection is obtained from an additive composition in which the carboxylic groups of the dicarboxylic acid component are in a plane symmetrical configuration. In the case of the stereo-isomeric acids, this configuration is easily recognizable as the cis form of the acid. As examples of the types of acids falling within this classification are the alkylated phthalic acid, alkylated hexahydrophthalic acid, alkyl malonic acid, alkyl maleic acid, and alkyl citraconic acid.

In its preferred form the invention contemplates a dicarboxylic acid obtained by the condensation of an olefin with maleic acid anhydride followed by hydrolysis. The condensation is carried out with an olefin, or mixtures thereof, either straight or branched chain containing an average of at least six carbon atoms and preferably ten or more. These olefins may be obtained from any of the usual sources, such as vapor phase cracking of petroleum oil or wax, or the polymerization of lower molecular weight olefins. The acids produced in this manner may exist as an alkyl maleic acid, an alkenyl succinic acid, or mixtures thereof. In order to simplify the description of these condensation products and the acids produced thereby, reference will be made throughout the specification and claims to alkyl maleic acids.

The second component of the additive composition, namely, the organic acid ester of an acid of phosphorus, embraces any organic ester of a phosphorus acid which contains at least one replaceable hydrogen linked to the phosphorus through an oxygen atom, and particularly the higher molecular weight organic esters which are soluble or miscible in the hydrocarbon or lubricating compositions. The acids of phosphorus whose organic acid esters satisfy the requirements of the present invention are the various phosphoric acids, which include the ortho, meta and pyro acids, together with the polymeric forms thereof. The organic esters of these acids may be the alkyl, aralkyl, aryl, and cycloalkyl esters, or mixtures thereof, which may be present as a mono- or di-ester, depending upon the available replaceable hydrogen present in the phosphorus acid. It is particularly desirable that these esters be sufficiently aliphatic in nature and of such molecular weight as to render the compound either oil-soluble or oil-miscible. Examples of the type of compounds falling within this classification which have been found satisfactory for use in the additive composition are the following: di-lauryl acid pyro-phosphate, n-butyl oleyl ortho-phosphate, mono-lauryl ortho-phosphate, and cresyl octyl acid ortho-phosphate.

In the preferred additive compositions of this invention the previously-mentioned alkyl maleic acid is combined with a high molecular weight alkyl acid phosphate which contains a total of at least 10 carbon atoms in the ester radicals thereof. These alkyl acid phosphates may be prepared by any of the known methods of synthesis and may consist of mixed alkyl esters, such as butyl lauryl acid ortho-phosphate or mixtures of mono- and di-substituted esters, such as mono- and di-lauryl acid ortho-phosphate, as well as the simple esters, such as mono-lauryl acid ortho-phosphate.

The amounts of the individual components of the additive composition to be incorporated in the hydrocarbon oil or lubricant will vary in accordance with the degree of rust protection and oxidation-resistant properties required. As a general proposition the dicarboxylic acid may be incorporated in ranges between 0.005 and 3.0% by weight, and the organic acid ester of an acid of phosphorus in ranges between 0.0001 and 2.5% by weight. In certain types of oils whose specifications include a maximum neutralization number, such as in turbine oil, the amounts of the acidic combination incorporated will necessarily have to be quite small. However, in other lubricating oils or compositions, where the neutralization number is not a serious factor and performance is the sole consideration, greater amounts of the additive composition may be incorporated.

As an added consideration of this invention, it has been found that foaming difficulties are encountered when the rust and oxidation-inhibited lubricating oils are used in certain circulatory or restricted lubricating systems, which are necessitated by recent developments in the design of internal combustion engines and other power plants where space is limited. This propensity toward foaming results in excessive frothing of the oil in the system, thus causing loss of lubrication and increased consumption of the oil.

According to a modification of the invention, it has been discovered that the foam-forming tendencies of a rust and oxidation-inhibited lubricating oil, such as the compounded oils of the present invention, may be retarded or minimized by the incorporation of a small amount of an organic silicone, such as dimethyl silicone polymer. These organic silicones may be obtained by hydrolysis of the di-alkyl or mixed alkyl-aryl silicon di-chlorides, prepared by a Grignard reaction using alkyl or mixtures of alkyl and aryl magnesium bromides and silicon tetra-chloride, and the silicons thus formed dehydrated by heat treatment. The resulting products are usually a mixture of the polymeric silicones and condensed silicons which have not been completely dehydrated. This product may be further polymerized by additional heat treatment, and organic silicones of varying degrees of polymerization and molecular weight may be obtained by varying the time and temperature of the heat treatment.

The organic silicones, and particularly the dimethyl silicones, are usually oil-insoluble and are incorporated in the lubricating oil by forming a kerosene solution thereof and incorporating the kerosene-silicone concentrate in the oil. To obtain foam-inhibiting properties very small amounts of the silicone need be incorporated in the oil and these amounts usually range between 0.00005% to 0.01% by weight of the silicones in the lubricating oil.

The results of numerous tests which are presented herein clearly illustrate the rust, oxidation

and foam-inhibiting properties of the oils compounded in accordance with the present invention. As illustrative of the increased oxidation-resistant properties obtained by the oxidation-inhibited oils compounded with the additive composition of the invention, the results obtained in the proposed ASTM oxidation test are presented. In this test, 300 ccs. of the oil sample are introduced to an oxidation cell in which is suspended spiral coils of iron and copper wire, and 60 ccs. of distilled water are added. Oxygen is introduced through a fritted glass outlet into the oxidation cell at the rate of 3 liters per hour. The oxidation cell is suspended in a heated oil bath and the temperature in the oxidation cell is maintained at a constant temperature of 95° C. Samples of the oil are periodically withdrawn to determine the neutralization number and the test continued until a neutralization number of 2 is obtained.

The reference oil used in this test was a solvent-refined acid-treated and filtered lubricating oil within the viscosity range of 485-515 Saybolt Universal at 100° F. To the reference oil were added varying amounts of accepted oxidation inhibitors and the resulting oxidation inhibited oils were then compounded with the additive composition of the present invention. For the purpose of this test the additive composition consisted of the combination of an alkyl maleic acid and an alkyl acid phosphate. The alkyl maleic acid was prepared by the condensation of maleic acid anhydride and a polymer gasoline distillate, boiling range 392-450° F. The reaction was obtained by heating with agitation for 20 hours and maintaining the liquid at a gentle reflux. Initial temperature 358° F., final temperature 390° F. After the heating was complete the reaction product was allowed to cool and fractionated under diminished pressure to remove unreacted polymer and low boiling reaction products. The alkyl maleic acid anhydride was then heated at about 200° F. in the presence of an equal volume of water until hydrolysis was complete and excess water had evaporated. The resulting alkyl maleic acid possessed a Neutralization No. of 336. The second component, namely, the alkyl acid phosphate was a commercial product consisting of a mixture of a mono- and di-lauryl acid ortho-phosphate which possessed an average Neut. No. of approximately 264 and contained an average of about 9.3% phosphorus.

ties of the oxidation-inhibited oil, compounded with the additive composition of the invention, is substantially greater than that obtained by the oxidation-inhibited oil, per se.

- 5 Additional test results have indicated that oils inhibited with other well-known oxidation inhibitors may also be improved by the addition of the combination of a dicarboxylic acid and an organic acid ester of an acid of phosphorus. 10 Among the specific compounds whose oxidation-inhibiting powers may be improved are the following:

Tetraethylamino diphenyl methane  
15 Di-isoamyl diaminodiphenyl methane  
Phenyl-alpha-naphthylamine thiocyanate  
Alpha, alpha-dinaphthylamine  
Alpha, beta-dinaphthylamine  
Beta, beta-dinaphthylamine  
Ortho-hydroxy benzyl alcohol  
20 Resorcinol mono-methyl ether  
Beta-naphthol disulfide  
Dibenzyl tetra sulfide  
2,2'-diaminodiphenyl disulfide  
25 Diethyl dithio oxalate  
Benzyl diethyl dithiocarbamate  
Zinc methyl cyclohexyl thiophosphate  
Dimethylaniline-sulfur reaction product  
Phenyl mercapto quinone  
30 Sulfurized beta-naphthol  
Sulfurized phenyl-alpha-naphthylamine  
Tetramethyl diaminodiphenyl disulfide  
Diphenyl mercaptol dibutyl ether

Furthermore, instead of the particular combination of components used in the additive composition in the test, other dicarboxylic acids, and particularly alkylated maleic acids obtained from olefins of higher or lower molecular weight may be used in combination with other organic acid esters of an acid of phosphorus, such as isoamyl octyl acid ortho-phosphate and dilauryl acid pyrophosphate.

The rust or corrosion-inhibiting properties of the oils compounded with the additive composition may be illustrated by the results obtained in a modified ASTM rusting test, using synthetic sea-water. In this test a polished steel specimen is suspended in an agitated mixture of 300 ccs. of the oil to be tested, and 30 ccs. of a synthetic sea-water. The oil sea-water sample is maintained at 140° F. over an oil bath for 48 hours, after which time the steel specimen is removed, allowed to drain, and washed with precipitation

#### Oxidation test

| Anti-Oxidant                                 | Per Cent | Additive Composition                         | Per Cent             | Hrs. to 2.0<br>Neut. No. |
|----------------------------------------------|----------|----------------------------------------------|----------------------|--------------------------|
| Ref. Oil                                     |          |                                              |                      |                          |
| Ref. Oil + Tetramethylamino diphenyl methane | 0.2      |                                              |                      | 65-72                    |
| Ref. Oil + Beta-naphthol                     | 0.2      |                                              |                      | 300                      |
| Ref. Oil + Butyl beta-naphthol               | 0.1      |                                              |                      | 174                      |
| Ref. Oil + Tetra amyl thiuram disulfide      | 0.2      |                                              |                      | 100                      |
| Ref. Oil                                     | +        | (Alkyl maleic acid<br>Lauryl acid phosphate) | 0.03<br>0.005 } (1)  | 250<br>140               |
| Ref. Oil                                     | +        | (Alkyl maleic acid<br>Lauryl acid phosphate) | 0.01<br>0.0025 } (2) | 80                       |
| Ref. Oil Tetramethylamino diphenyl methane   | 0.2+     | (Composition 2)                              |                      | 1399                     |
| Ref. Oil Beta-naphthol                       | 0.2+     | (Composition 1)                              |                      | 740                      |
| Do.                                          | 0.2+     | (Composition 2)                              |                      | 300                      |
| Ref. Oil Butyl beta-naphthol                 | 0.4+     | do                                           |                      | 150                      |
| Ref. Oil Phenyl alpha-naphthylamine          | 0.2+     | do                                           |                      | 570                      |
| Do.                                          | 0.4+     | do                                           |                      | 897                      |
| Ref. Oil Phenyl beta-naphthylamine           | 0.4+     | do                                           |                      | 1.6                      |
| Ref. Oil Tetra amyl thiuram disulfide        | 0.2+     | do                                           |                      | 250                      |
| Ref. Oil Acetone diamyl mercaptol            | 0.2+     | do                                           |                      | 315<br>290               |

It may be seen from the results obtained that in each instance the oxidation-resistant proper-

naphtha or hexane and the amount of corrosion or rust observed.

The synthetic sea-water added to the test oil is made up of the following composition:

|                                             | Gm. per liter |
|---------------------------------------------|---------------|
| Magnesium chloride ( $MgCl_2 \cdot 6H_2O$ ) | 11.0          |
| Anhydrous calcium chloride ( $CaCl_2$ )     | 1.2           |
| Anhydrous sodium sulphate ( $Na_2SO_4$ )    | 4.0           |
| Sodium chloride ( $NaCl$ )                  | 25.0          |

The reference oil and the components of the additive composition used in this test were the same as previously described for the oxidation test. The results obtained are as follows:

| 5                      | Element | Analysis, percent |
|------------------------|---------|-------------------|
| Carbon                 |         | 32.35             |
| Hydrogen               |         | 8.15              |
| Silicon                |         | 38.50             |
| Oxygen (by difference) |         | 23.00             |

10 When 0.0001% by weight of the dimethyl silicone polymer was added to the compounded oil

| Anti-Oxidant                                    | Percent | Additive Composition   | Percent | Appearance of Steel Specimen |
|-------------------------------------------------|---------|------------------------|---------|------------------------------|
| Ref. Oil                                        |         |                        |         | Heavy Rust.                  |
| Ref. Oil + Tetramethyl diamino diphenyl methane | 0.1     | [Alkyl maleic acid     | 0.03    | Do.                          |
| Ref. Oil Tetramethyl diamino phenylmethane      | 0.2+    | [Lauryl acid phosphate | 0.005   | Clean.                       |
| Ref. Oil Tetramethyl diamino diphenyl methane   | 0.2+    | [Alkyl maleic acid     | 0.01    | Do.                          |
| Ref. Oil Beta-naphthol                          | 0.2+    | [Lauryl acid phosphate | 0.0025  | Do.                          |
| Do                                              | 0.2+    | [Alkyl maleic acid     | 0.03    | Do.                          |
| Ref. Oil Phenyl alphanaphthylamine              | 0.2+    | [Lauryl acid phosphate | 0.005   | Do.                          |
| Do                                              | 0.4+    | [Alkyl maleic acid     | 0.01    | Do.                          |
| Ref. Oil Tetra amyl thiuram disulfide           | 0.2+    | [Lauryl acid phosphate | 0.0025  | Do.                          |
| Ref. Oil Acetone diamyl mercaptol               | 0.2+    | [Alkyl maleic acid     | 0.01    | Do.                          |
|                                                 |         | [Lauryl acid phosphate | 0.0025  | Do.                          |

Although the oils compounded in accordance with the present invention have been shown to possess excellent oxidation and rust-inhibiting properties, there remains another factor to be considered before the compounded oils can be successfully used in operation in certain types of modern power plants. This factor is a tendency of the oil to foam in restricted lubricating systems. As previously mentioned, these rust and oxidation-inhibited oils may be further inhibited against foaming by the addition of an organic silicone, such as a dimethyl silicone polymer. The following tests have been designed to determine the tendency of lubricating oil foam, which is produced by mechanical agitation in the presence of air, to break and return to the oil phase:

200 grams of the test oil are weighed into an 800 cc. beaker and brought up to a temperature of 120° F. After reaching the test temperature, the oil is agitated for three minutes with a double-paddle mechanical stirrer operating at a constant speed of 980-1000 R. P. M. Thereafter, the stirrer paddles are allowed to drain for fifteen seconds and the contents of the beaker poured quickly into a 500 cc. graduated cylinder. While maintaining the oil in the graduate at 120° F., the volume of oil plus foam and clear oil is read at ten minute intervals for 60 minutes, and the volume of foam is determined as the difference between the two readings.

In this test the reference oil used was a solvent-refined, acid-treated and filtered lubricating oil within the viscosity range of 418-515 S. U. at 100° F. This oil was then compounded with 0.01% alkyl maleic acid (prepared in accordance with the example given for the oxidation test), 0.0025% lauryl acid phosphate and 0.2% tetramethyl diamino diphenyl methane. The results obtained showed 225 ccs. of foam at 60 minutes, with a duplicate run showing 235 ccs. of foam at 60 minutes. To this test oil were then added varying amounts of an organic silicone polymer. The particular polymer used was a dimethyl silicone polymer which consisted substantially of

35 the results showed no foam at 60 minutes. When 0.002% by weight of the dimethyl silicone was added the results indicated no foam at ten minutes.

40 Obviously many modifications and variations of the invention, as hereinbefore set forth, may be made without departing from the spirit and scope thereof, and therefore only such limitations should be imposed as are indicated in the appended claims.

We claim:

45 1. A lubricating oil composition having superior anti-oxidant and anti-rusting properties in the presence of water comprising as essential ingredients a hydrocarbon oil possessing lubricating properties and having incorporated therein about 0.01-5.0% by weight, on the basis of the lubricating composition, of an alkyl substituted diamino diphenyl methane, about 0.005-3.0% by weight of an oil-miscible dicarboxylic acid having at least 10 carbon atoms in the molecule and a plane symmetrical configuration, and about 0.0001-2.5% by weight of an oil-miscible 50 55 alkyl acid phosphate containing at least 10 carbon atoms in the alkyl portion thereof.

60 2. A lubricating oil composition having superior anti-oxidant and anti-rusting properties in the presence of water comprising as essential ingredients a mineral lubricating oil having incorporated therein about 0.1-2.0% by weight of tetramethyl diamino diphenyl methane, about 0.005-3.0% by weight of an oil-miscible alkyl maleic acid having at least 10 carbon atoms in the molecule, and about 0.0001-2.5% by weight of an oil-miscible alkyl acid phosphate having at least 10 carbon atoms in the ester portion thereof.

65 70 3. A lubricating oil composition having superior anti-oxidant and anti-rusting properties in the presence of water comprising as essential ingredients a mineral lubricating oil having incorporated therein about 0.1-0.2% by weight of tetramethyl diamino diphenyl methane, about 0.01-0.03% by weight of an alkyl maleic acid, 75 which is the hydrolyzed condensation product of

maleic anhydride with a polymer gasoline distillate, and having at least 10 carbon atoms in the molecule, and about 0.0025-0.005% by weight of a lauryl acid orthophosphate.

4. A lubricating oil composition according to claim 3, wherein the mineral lubricating oil also has incorporated therein about 0.0001-0.002% by weight of an oil-insoluble alkyl silicone polymer.

JOHN A. PATTERSON. 10  
HERMAN D. KLUGE.

## REFERENCES CITED

The following references are of record in the file of this patent:

## UNITED STATES PATENTS

| Number       | Name      | Date          |
|--------------|-----------|---------------|
| 2,080,299    | Benning   | May 11, 1937  |
| 2,129,281    | Lincoln   | Sept. 6, 1938 |
| 5 2,133,734  | Moser     | Oct. 18, 1938 |
| 2,157,873    | Van Peski | May 9, 1939   |
| 2,226,543    | Ashburn   | Dec. 31, 1940 |
| 2,258,218    | Rochow    | Oct. 7, 1941  |
| 2,265,962    | Bent      | Dec. 9, 1941  |
| 10 2,315,072 | Nelson    | Mar. 30, 1943 |
| 2,323,670    | Musselman | July 6, 1943  |
| 15 2,324,577 | Haffner   | July 20, 1943 |
| 2,334,158    | Von Fuchs | Nov. 9, 1943  |
| 2,346,357    | Burk      | Apr. 11, 1944 |
| 2,375,007    | Larsen    | May 1, 1945   |